# EUROPEAN PATENT SPECIFICATION

(11) **EP 0 090 118 B1**
(45) Date of publication and mention of the grant of the patent: **05.03.1986**
(21) Application number: 82306346.6
(22) Date of filing: 30.11.1982
(51) Int. Cl.: B22C 3/00, B22C 9/00, B22C 13/08, B22F 3/00

(54) **Ceramic mould and method of producing same**
Keramikform und Verfahren zur Herstellung derselben
Moule céramique et procédé pour la production de celui-ci

(30) Priority: 26.03.1982 US 362341
(43) Date of publication of application: 05.10.1983
(73) Proprietor: CRUCIBLE MATERIALS CORPORATION, Syracuse, New York 13201-0977 (US)
(72) Inventor: Chandhok, Vijay Kumar, Allegheny Pennsylvania 15228 (US); Brosius, Karl Simms, Washington Pennsylvania 15021 (US); McCollough, William Lee, Allegheny Pennsylvania 15044 (US)
(74) Representative: Sheader, Brian N.

## Description

This invention relates to ceramic moulds and to a method of producing same.

It is known to produce powder metallurgy shapes of various configurations by the use of a ceramic shell-type mould. The ceramic mould has an interior which conforms to the desired configuration of the article to be produced. The cavity is filled with powdered metal, the mould is sealed, heated and then subjected to force sufficient to compact the powdered metal therein to form a dense article. The preferred compacting method is to place the powder filled mould at elevated temperature in an autoclave for hot isostatic pressing by the use of a gas, such as helium.

One practice for producing moulds of this type involves making a wax pattern of the configuration of the article to be produced and then casting the ceramic around the pattern so that the interior of the ceramic conforms to the surface configuration of the pattern and thus the article to be produced. An opening is provided in the ceramic through which upon heating the wax may be melted to expose the cavity. Thereafter the cavity is filled with powdered metal and the powder is compacted in the conventional manner as by hot isostatic compacting.

In operations of this type, during heating of the powder within the ceramic mould the powder tends to become contaminated by the ceramic with which which it is in contact within the mould cavity. Particles of the ceramic, including oxides, enter the powder and during compacting are confined within the densified article. These non- metallic substances weaken the article such as by providing sites for crack propogation. In addition, reaction products, which be from the ceramic, chemically react with powder metal to form non- metallic compounds at prior particle boundaries after compacting.

It is accordingly a primary object of the present invention to provide a ceramic mould adapted for use in producing powder metallurgy articles of intricate configuration that avoids contamination of the metal article by contact with the ceramic material.

Broadly, according to the present invention there is provided a ceramic mould body having a mould cavity therein with the surface of the mould cavity conforming substantially to the configuration of the article to be produced. The mould cavity is generally somewhat "oversize" with respect to the final article to allow for shrinkage during compacting. An opening is provided for filling the cavity with powdered metal and thereafter sealing it prior to compacting. In accordance with the invention the mould cavity has a continuous metal coating covering its surface. This prevents contact between the metal powder and the ceramic material of the mould and thus acts as a barrier to prevent contamination by impurities such as oxides from entering the powder during the heating and compacting cycle. A preferred material for this coating is nickel or nickel-base alloys as they remain continuous during the high temperatures incident to hot compacting operations such as hot isostatic pressing. In accordance with the invention, the alloy powders are generally superalloys, such as nickel, iron or cobalt-base alloys, and titanium- base alloys for use in high temperature applications, such as jet engine components and the like. However, the mould of the invention is also suitable for use with high speed steels and tool steels. Preferably, to facilitate coating of the mould cavity surface the mould is segmented into at least two selectively separated parts. When separated the interior can be coated with the metal and then the parts can be joined to form the integral mould. A preferred method for applying the coating so that it is thin and continuous involves vapour deposition.

It is known to produce powder metallurgy articles that have, after compacting, internal passages. This is conventionally achieved by providing within the mould a ceramic core or mandrel having an exterior configuration conforming to that of the internal passage desired to be produced in the final compacted article. The powder fills the mould and surrounds the mandrel. During compacting, the powder is compacted against the mandrel, and upon removal of the mandrel after compacting an internal passage is produced within the compacted article. To produce an article with an internal passage, in accordance with the present invention, the exterior of the core or mandrel is coated with metal to prevent contamination of the powder.

The invention will be more particularly described with reference to the accompanying drawings, in which:-
Figure 1 is a cross-section of one embodiment of a mould according to the present invention.
Figure 2 is a cross-section of the mould of Figure 1 having the mould cavity filled with metal powder and being ready for compacting;
Figure 3 is an elevation of a powder metallurgy product resulting from compacting using the mould of Figures 1 and 2; and
Figures 4, 5 and 6 are photomicrographs at a magnification of 150x showing compacted alloys produced by the use of conventional ceramic moulds and moulds according to the present invention.

With respect to the drawings, Figure 1 shows two identical mould segments in cross-section identified as 10 having a ceramic body portion 12 with a mould cavity 14 conforming to the configuration of the article to be produced, which in this case is a gearwheel. The gear teeth 16 are defined in the interior surface of the body 12. This may be achieved by dipping a wax pattern conforming substantially to the shape of the gear wheel in a refractory slurry and then melting away the wax after drying the refractory material. Although this method is preferred, any other method may be used for producing the mould. The interior surfaces of the mould cavity are coated with a metal 18, as shown in Figure 2, and the segments are joined and filled with powdered metal 20. The mould is then sealed and compacted such as by hot isostatic compacting. Upon removal of the compacted article, the gear, designated as 22, is produced as shown in Figure 3. Although the terms "metal", "nickel" and "titanium" are used herein it is to be understood that these include alloys as well as metal in elemental form.

The following specific examples are illustrative of the present invention:

### Example I

A ceramic shell was internally coated with nickel using the chemical vapour deposition (CVD) process. This involved injecting nickel carbonyl gas into the heated shell, whereupon the nickel metal was deposited by thermal decomposition of the gas onto the surface of the shell cavity. A coating was produced with certain areas left bare. The coating thickness was of the order of 0.0254 to 0.254 mm (1 to 10 mils). The shell was then processed in a normal manner to produce a powder metallurgy part, using a conventional nickel-base superalloy powder (Rene 95). The resulting compact was normal with an unusually bright surface appearance. Metallographic examination revealed a nickel surface coating, a boundary layer of interdiffusion products, and the Rene 95 base metal (see Figure 4). In an area unprotected by the nickel coating, the Rene 95 powder particles are outlined by a contamination layer, a normal phenomenon with the conventional ceramic mould process (see Figure 5). The nickel coating is thus seen to provide protection for contamination for the Rene 95 base metal from which the final compacted superalloy is to be made.

### Example 11

A ceramic shell was split and the interior of the shell conforming to the powder metallurgy article to be produced was coated with nickel by the ion deposition process wherein metal atoms are directly deposited on the target surface in a vacuum chamber. The coating thickness was of the order of 0.00254 mm (.1 mils). The shell was then processed in a normal manner to produce a powder metallurgy part, using titanium alloy powder. This included filling the shell with titanium alloy powder, evacuating, heating and hot-isostatic pressing to compact the powder to full density. The resulting compact had an unusually smooth surface appearance. Metallographic examination revealed a surface diffusion-products layer of the order of 0.00254 mm (.1 mil) thick (see Figure 6).

In addition to the metal coating techniques demonstrated in the specific examples, a metal coating may be produced on the interior surfaces of a ceramic shell such as by electroplating the metal coating, which may be nickel, on a wax pattern shape and then providing a ceramic shell around this metal-coated wax pattern, as by dipping the assembly in a refractory slurry. When the wax is removed by melting followed by chemical cleaning the metal layer remains bonded to the ceramic shell to produce the desired shell mould with a metal coated interior. A wax pattern may be coated with nickel by first spraying the surface of the pattern with graphite to provide an electrically conductive base and then electroplating onto this conductive base a metal such as nickel.

## Claims

1. A mould (10) for use in the production of a powder metallurgy article (22), comprising a ceramic mould body (12) having a mould cavity (14) therein with a surface conforming substantially to the configuration of a said article to be produced and adapted for filling with a powdered metal (20) for compaction to form said article, characterised in that said mould cavity (14) has a continuous metal coating (18) covering said surface.

2. A mould according to claim 1, characterised in that said metal coating (18) is nickel.

3. A mould according to claim 1 or 2, characterised in that said ceramic mould body (12) is segmented into at least two selectively separable parts.

4. A mould according to claim 1, 2 or 3, characterised in that said mould (10) has a ceramic core within said mould cavity (14) an said ceramic core has a continuous metal coating thereon.

5. A method of producing a mould (10) for use in the production of a powder metallurgy article (22), said method comprising producing a ceramic mould body (12) having a mould cavity (14) therein with a surface conforming substantially to the configuration of said article (22) and adapted for filling with powdered metal (20) for compaction to form said article (22), characterised in that the method further comprises applying a continuous metal coating (18) onto said surface.

6. A method according to claim 5, characterised in that said ceramic mould body (12) is produced by forming at least two separable segments (10) and uniting said segments to result in said mould cavity (14).

7. A method according to claim 6, characterised in that said segments (10) each have a surface portion adapted to form said mould cavity (14) when said segments (10) are united and a continuous metal coating (18) is applied to said surface portion prior to uniting said segments (10) to result in said mould cavity (14).

8. A method according to claim 5, 6 or 7, characterised in that said metal coating (18) comprises nickel.

9. A method according to any one of the preceding claims 5 to 8, characterised in that said coating (18) is applied by chemical vapor deposition.

10. A method according to any one of the preceding claims 5 to 9, characterised in that a ceramic core having a continuous metal coating thereon is provided within said mould cavity.

## Patentansprüche

1. Form (10) für die Herstellung von pulvermetallurgischen Artikeln (22), die einen Keramikformkörper (12) mit einem inneren Hohlraum (14) aufweist, dessen Oberfläche der äußeren Form des herzustellenden Artikels entspricht und der mit einem Metallpulver (20) ausfüllbar ist, aus dem durch Verpressen der Artikel geformt wird, dadurch gekennzeichnet, daß der Hohlraum (14) der Form eine lückenlose Metallbeschichtung (18) aufweist, die die Hohlraumoberfläche bedeckt.

2. Form nach Anspruch 1, dadurch gekennzeichnet, daß die Metallbeschichtung (18) aus Nickel ist.

3. Form nach Anspruch 1 oder 2, dadurch gekennzeichnet, daß der Keramikformkörper (12) in zumindest zwei einzelne separate Teile aufgeteilt ist.

4. Form nach Anspruch 1, 2, oder 3, dadurch gekennzeichnet, daß die Form einen Keramikkern innerhalb des Hohlraums (14) der Form aufweist, und daß der Keramikkern eine lückenlose Metallbeschichtung aufweist.

5. Verfahren zur Herstellung einer Form (10) für die Verwendung bei der Herstellung eines pulvermetallurgischen Artikels (22), wobei ein Keramikformkörper (12) mit einem inneren Hohlraum (14) hergestellt wird, dessen Oberfläche der äußeren Form des Artikels (22) entspricht und in den Metallpulver zur Verpressung und Formung des Artikels (22) einfüllbar ist, dadurch gekennzeichnet, daß in einem weiteren Verfahrensschritt eine lückenlose Metallbeschichtung (18) auf die Oberfläche des Hohlraumes (14) aufgebracht wird.

6. Verfahren nach Anspruch 5, dadurch gekennzeichnet, daß der Keramikformkörper (12) aus zumindest zwei separaten Segmenten (10) hergestellt wird und daß die Segmente zur Bildung des Hohlraumes (14) zusammengefügt werden.

7. Verfahren nach Anspruch 6, dadurch gekennzeichnet, daß die Segmente (10) jeweils einen Oberflächenteil aufweisen, aus dem der Hohlraum (14) gebildet wird, wenn die Segmente (10) zusammengefügt sind, und daß eine lückenlose Metallbeschichtung (18) auf diesen Oberflächenteil aufgebracht wird, bevor diese Segmente (10) zur Bildung des Hohlraumes (14) zusammengefügt werden.

8. Verfahren nach Anspruch 5, 6 oder 7, dadurch gekennzeichnet, daß die Metallbeschichtung (18) Nickel enthält.

9. Verfahren nach einem der vorhergehenden Ansprüche 5 bis 8, dadurch gekennzeichnet, daß die Beschichtung (18) mit Hilfe chemischer Gasphasenabscheidung aufgebracht wird.

10. Verfahren nach einem der vorhergehenden Ansprüche 5 bis 9, dadurch gekennzeichnet, daß innerhalb des Hohlraums der Form ein Keramikkern mit einer lückenlosen Metallbeschichtung vergesehen wird.

## Revendications

1. Moule (10) destiné à être utilisé pour produire par la métallurgie des poudres un objet (22), comprenant un corps de moule céramique (12), à l'intérieur duquel se trouve une cavité de moule (14) dont la surface se conforme pratiquement à la configuration de l'objet à produire et qui est adaptée pour être remplie par un métal en poudre (20) pour subir un compactage pour former cet objet, caractérisé en ce qu'un revêtement métallique continu (18) recouvre la surface de la cavité du moule (14).

2. Moule selon la revendication 1, caractérisé en ce que ce revêtement métallique (18) est du nickel.

3. Moule selon la revendication 1 ou la revendication 2, caractérisé en ce que le corps (12) du moule céramique est segmenté en au moins deux parties sélectivement séparables.

4. Moule selon l'une des revendications 1, 2 ou 3, caractérisé en ce que ce moule (10) a un noyau céramique à l'intérieur de la cavité de moule (14) et qu'un revêtement métallique continu est déposé sur ce noyau céramique.

5. Procédé pour produire une moule (10) destiné à être utilisé pour produire, par la métallurgie des poudres, un objet (22), ce procédé consistant à produire un corps de moule céramique (12) à l'intérieur duquel se trouve une cavité de moule (14) dont la surface se conforme pratiquement à la configuration de l'objet (22) et qui est adaptée pour être remplie d'un métal en poudre (20) pour subir en compactage pour former cet objet (22), caractérisé en ce que ce procédé consiste en outre à appliquer un revêtement métallique continu (18) sur cette surface.

6. Procédé selon la revendication 5, caractérisé en ce que ce corps de moule céramique (12) est produit en formant au moins deux segments séparables (10) et en raccordant ces segments pour obtenir la cavité de moule (14).

7. Procédé selon la revendication 6, caractérisé en ce que chacun de ces segments (10) a une portion de surface adaptée pour former la cavité de moule (14) lorsque ces segments (10) sont raccordés et en ce qu'un revêtement métallique continu (18) est appliqué sur cette portion de surface avant raccordement des segments (10) pour obtenir la cavité de moule (14).

8. Procédé selon l'une des revendications 5, 6 ou 7, caractérisé en ce que ce revêtement métallique (18) est du nickel.

9. Procédé selon l'une quelconque des revendications 5 à 8 précédentes, caractérisé en ce que ce revêtement (18) est appliqué par dépôt chimique en phase vapeur.

10. Procédé selon l'une quelconque des revendications 5 à 9 précédentes, caractérisé en ce qu'un noyau céramique, sur lequel est déposé un revêtement métallique continu, est prévu à l'intérieur de la cavité du moule.
